

992,463.

L. P. WHITAKER.  
PROCESS FOR MANUFACTURE OF STEEL RINGS.  
APPLICATION FILED APR. 20, 1910.

Patented May 16, 1911.

FIG. 1.



FIG. 2.



FIG. 3.



WITNESSES

*J. F. Taylor*  
J. K. Moore

INVENTOR

*Louis P. Whitaker*  
BY

*Whitaker & Proctor*

Attorneys

# UNITED STATES PATENT OFFICE.

LOUIS P. WHITAKER, OF WASHINGTON, DISTRICT OF COLUMBIA, ASSIGNOR TO S. R. DRESSER MANUFACTURING COMPANY, OF BRADFORD, PENNSYLVANIA, A CORPORATION OF PENNSYLVANIA.

## PROCESS FOR MANUFACTURE OF STEEL RINGS.

992,463.

Specification of Letters Patent. Patented May 16, 1911.

Application filed April 20, 1910. Serial No. 556,542.

*To all whom it may concern:*

Be it known that I, LOUIS P. WHITAKER, a citizen of the United States, residing at Washington, in the District of Columbia, 5 have invented certain new and useful Improvements in Processes for the Manufacture of Steel Rings; and I do hereby declare the following to be a full, clear, and exact description of the invention, such as 10 will enable others skilled in the art to which it appertains to make and use the same.

My invention consists in a process for the manufacture of rings from steel or other wrought metal, and particularly for the 15 manufacture of steel clamping rings for rubber packed pipe couplings, and said invention is illustrated in the accompanying drawing forming part of this specification and is fully disclosed in the following description and claims.

In the accompanying drawing, Figure 1 represents a blank for the ring. Fig. 2 represents the blank bent into ring form preparatory to welding. Fig. 3 represents a 20 section of the completed ring.

The object of my improved process is to produce a wrought metal ring (preferably of steel) in which the molecules are in an inequiaxed condition, thus setting up internal stress and raising the yield point of the 30 metal of the ring and producing a ring which will stand much greater stress before yielding than a ring of the same size and cross section formed of metal in which the molecules are in the ordinary or equiaxed condition.

In carrying out my invention I first produce a bar of substantially the cross section which is desired in the finished ring. The 40 clamping ring which it is the special object of my improved process to produce, is provided with an annular flat member, which I term for convenience of reference, the plate member, and from which an annular flange member extends on one side of the plate member, the said flange member having its base located between the inner and outer edges of the plate member. In carrying out the first step of the process I, 45 therefore, first produce a bar, having in this instance a flat plate member, and a perpendicular flange extending from one side of the same, and located between the lateral edges of the plate member, thus hav-

ing in cross section something of the appearance of an inverted letter T. In Fig. 1, I have shown such a bar, the plate member of which is indicated at 1, and the flange member of which is indicated at 2. In practice the flange 2 is located nearer that edge of the plate member which is to form the inner edge of the ring, here indicated at 3 and the plate member is preferably made slightly thicker adjacent to the edge 3 than it is adjacent to the opposite edge 4, 55 and preferably diminishes slightly in thickness from the intermediate flange member 2 toward the edge 4. This bar may be formed in any one of several ways, as by rolling it in the desired form, or by planing it to the 60 desired form, or in other ways which will suggest themselves to the skilled mechanic. The previously formed bar is then cut to the desired length, such as when bent into ring form, will produce a ring of the desired 65 diameter. The bar or blank so formed is then bent into ring form in the plane of the plate member 1 thereof, below such temperature as will permit the molecules of the 70 metal which will be forced into an inequiaxed condition by the bending operation, to return to the equiaxed condition and thereby certain internal strains are set up within the bar. It is known that above a 75 certain temperature, which for convenience 80 may be herein designated the "critical temperature" and which may be described with sufficient definiteness as a "red heat visible in daylight", the molecules of steel remain equiaxed (or having all their axes equal), 85 during the changes in the form of the material. If, however, a bending operation for example is performed upon a bar of steel at any temperature below the "critical temperature" the molecules of the metal become 90 inequiaxed, and internal stress is set up within the metal which raises the yield point, or elastic limit of the metal, and 95 greatly increases its stiffness.

The metal blank or bar may be bent or 100 formed into ring shape as before described by any suitable means, and the operation is preferably performed while the metal is at a temperature just below a visible red, although it may be performed while the metal 105 is cold, or at any temperature below the "critical temperature."

Fig. 2 represents the bar bent into the

shape of a ring, with its ends brought together for welding. As shown the meeting ends of the bar are cut at substantially right angles to the bar, for the purpose of forming 5 a butt weld, but they may be so formed as to produce a lap weld if desired. The welding operation itself is preferably performed electrically in a well known way so that only a small amount of the metal at each side of 10 the weld will be raised to or above the "critical temperature." It may, however, be performed otherwise, as by heating the meeting ends of the bar only, in a gas furnace, care being taken to raise a small portion only of 15 the ring at each side of the weld above the "critical temperature."

As the effect of raising portions of the metal adjacent to the weld above the "critical temperature" is to permit the molecules 20 thereof to return to an equiaxed condition, the portions of the ring so affected, are after the welding operation subjected to a compressing action or mechanical working, after the metal adjacent to the weld has cooled 25 below the "critical temperature," as by hammering or rolling after the metal has cooled below such "critical temperature." This working of the metal again inequiaxes the molecules of the portion of the metal which 30 was annealed during the welding operation, and again sets up a condition of internal stress therein, thus making the portions of the ring adjacent to the weld substantially as stiff as the other portions of the ring.

35 The resulting ring, which is illustrated in Fig. 3 of the drawing, will be found to have much greater stiffness than a ring of the same weight and thickness of metal which is made by operations conducted while the 40 metal is above the "critical temperature." The ring is finished by perforating the outer portion of the plate member while below the critical temperature (and preferably while cold) as at 5, 5 etc., to form bolt holes 45 to receive the coupling bolts of a pipe coupling. As will be seen the plate or base portion of the bar 1 forms the annular plate member 1<sup>a</sup> of the ring, and the flange member 2 of the bar forms the annular flange member 2<sup>a</sup> of the ring (the edge 3 of the bar

55 forming the inner edge 3<sup>a</sup> of the plate member of the ring and the edge 4 of the bar forming the outer edge 4<sup>a</sup> of the plate member of the ring). I have indicated the weld at 6 and by dotted lines 7, 7, the portions at 60 each side of the weld, which are annealed during the welding and are subsequently restored to an inequiaxed molecular condition by hammering or otherwise mechanically working the metal. In some instances I 65 may employ a rolling operation between specially formed rolls for the purpose of restoring the annealed portions of the ring after welding, to an inequiaxed molecular condition.

65 What I claim and desire to secure by Letters Patent is:—

1. The herein described process of producing a steel ring, which consists in forming a straight bar of steel of the desired 70 section, bending the bar into ring form, at a temperature which will raise the yield point of the metal, welding the meeting ends of the bar, and mechanically working the annealed portions of the bar adjacent to the 75 weld, after they cool below the "critical temperature" to raise the yield point thereof.

2. The herein described process of making a steel clamping ring for pipe couplings, 80 which consists in forming a bar of steel having a plate member and a perpendicularly disposed flange member, bending the bar in the plane of the plate member thereof into ring form, at a temperature which will raise the yield point of the metal, heating only 85 the portions of the bar adjacent to its meeting ends to a welding heat and welding the ends together, then mechanically working the portions of the ring heated above the "critical temperature" during the welding process, after they have cooled below said "critical temperature" to again raise the 90 yield point thereof.

In testimony whereof I affix my signature, in the presence of two witnesses.

LOUIS P. WHITAKER.

Witnesses:

J. K. MOORE,  
Wm. F. DOYLE.